

May 27, 1947.

F. M. CLARK

2,421,241

LIQUID-QUENCHED SWITCH

Filed Aug. 9, 1944



Inventor:  
Frank M. Clark,

by *Harry E. Dunham*  
His Attorney.

## UNITED STATES PATENT OFFICE

2,421,241

## LIQUID-QUENCHED SWITCH

Frank M. Clark, Pittsfield, Mass., assignor to  
General Electric Company, a corporation of  
New York

Application August 9, 1944, Serial No. 548,678

10 Claims. (Cl. 200—150)

1

The present invention relates to liquid-quenched make-and-break electrical devices, such as commonly known by the term "oil-filled" circuit breakers, contactors, cut-outs and the like.

Petroleum oil has most commonly been employed as the quenching liquid in such devices. However, petroleum oil is partially decomposed when subjected to contact with an electric arc or spark. As a consequence of the decomposition, carbon is set free and gas is evolved. The carbon remains in suspension in the oil and the gas escapes. The gradual accumulation of carbon in the liquid is troublesome and may lead to failures and breakdowns. The carbon tends to become deposited on the surfaces of the switch mechanism and interfere with its proper functioning. Electric short circuits may occur and, in general, electrical creepage effects reduce the efficiency of the apparatus. When the circuit interrupter or contactor operates in a sealed container, excessive pressure caused by the accumulation of gas therein may be dangerous. Attempts made heretofore to provide an improved arc-quenching liquid have not been successful.

The present invention is based on the discovery that the undesirable results obtained with petroleum oil, that is, the formation of carbon and its tendency to settle on the insulating and the contacting parts of the mechanism, are reduced or entirely eliminated when electric arcs are quenched by an alkyl ester of an organic acid. In other words, when properly chosen liquid organic esters are subjected to the electric arc as in a contactor or switch, they evolve greatly reduced quantities of carbon and gas. The carbon formed is in such physical state that it has substantially no tendency to settle. Properly selected liquid-quenching agents in devices embodying my invention produce only about 10 per cent of the amount of carbon normally formed under the same degree of use in mineral oil.

The accompanying drawing shows conventionally an electric contactor embodying my invention.

As shown in the drawing, the contact-making and breaking electrodes 1, 2 are mounted on a suitable support 3 consisting of insulating material within a tank or housing 4 containing a body 5 of quenching liquid. The contact 1 is yieldably supported on an arm 6 which is movably pivoted

2

on a bearing 7. A circuit conductor 8 has been indicated for carrying current to the contact 1. The contact 1 is brought into engagement with the contact 2 by a magnet (not shown) which is connected to a lever arm 9 whereby the movable contact is operated. The contact 2 is fixedly supported on a conductive bracket 10. When the operating magnet is deenergized, the contacts 1 and 2 are disengaged by gravity. The arcing contacts 1, 2 may comprise copper, silver or other suitable metal and may be confined, as shown, between shields 11, 12 consisting of insulating material. The enclosing housing 4 is supported by a hanger 13 from a fixed bracket 14. As switches of the liquid-quenched type are well known in the electrical field, the structural features of the device need not be described in greater detail.

The arc-quenching liquid 5 indicated in the drawing comprises one or more alkyl esters of organic acids from 2 to 18 carbon atoms, as for example the esters of stearic and oleic acids ( $C_{17}H_{35}COOH$  and  $C_{11}H_{23}COOH$ , respectively). The alkyl radicals associated with these acids contain preferably one to five carbon atoms and comprise the methyl, ethyl, propyl, butyl and amyl groups. The chosen ester should be insoluble in water, or substantially so, as otherwise it may pick up water with accompanying depreciation of insulating properties.

Illustrative of acid radicals which I have found of utility in accordance with my invention are the following: stearic, oleic, oxalic, ricinoleic, lauric, lactic, tartaric, sebatic, acetic, citric, propionic, caprylic and caproic acid.

Specific illustrations of alkyl esters suitable for the purposes of my invention are the following: butyl ricinoleate, glycol diricinoleate, 2-butoxyethanol,  $C_4H_9-O-CH_2-CH_2-OH$ , ricinoleate, 2-methoxyethanol ricinoleate, glycol dioleate, butyl oleate, amyl oleate, methyl oleate, butyl stearate, methyl stearate, butyl laurate, ethyl laurate, butyl tartrate, dibutyl sebacate, 2-ethyl hexyl sebacate, ethyl citrate, butyl citrate, 2-butoxyethanol citrate, butyl lactate, 2-ethoxyethanol acetate, ethyl levulinate, butyl oxalate, amyl oxalate, ethyl hydroxy propionate, butyl caproate and butyl caprylate. It will be observed that the alcoholic radicals of short chain length are combined with acid radicals of longer chain length and vice versa.

Although all of the ester compositions of my invention are characterized by substantially no carbon deposition on contacting or dielectric surfaces, thereby insuring freedom from electrical deterioration in use, and although all are characterized by a high and stable dielectric strength despite the most severe arcing in service use, it is nevertheless possible to classify dielectric ester compositions which are suitable for arc-quenching purposes as forming two distinct groups on the basis of the amount of carbon formed under identical conditions of arcing.

In the first group are the methyl, ethyl, propyl, butyl or amyl esters of the monocarboxylic acids such as:

Stearic ( $C_{17}H_{35}COOH$ )  
Oleic ( $C_{17}H_{33}COOH$ )  
Lauric ( $C_{11}H_{23}COOH$ )  
Acetic ( $CH_3COOH$ )  
Propionic ( $C_2H_5COOH$ )  
Caproic ( $C_5H_{11}-COOH$ )  
Caprylic ( $C_7H_{15}-COOH$ )

In general, this group includes the ester derivatives of the saturated and unsaturated carboxylic acids of the chain or aliphatic series as distinguished from the ring or benzenoid carboxylic acids.

In the second and preferred classification of ester arc-quenching compositions contained in apparatus embodying my invention may be grouped the methyl, ethyl, propyl, butyl and amyl esters of those organic acids which contain either a carboxylic group in combination with a hydroxy or ketone group or a plurality of carboxylic groups or both. Illustrative of such acids are the following:

Oxalic acid ( $COOH-COOH$ )  
Ricinoleic acid ( $C_{17}H_{32}(OH)COOH$ )  
Hydroxy propionic acid  $CH_3-CHOH-COOH$   
Sebacic acid ( $CH_2$ )<sub>8</sub>-( $COOH$ )<sub>2</sub>  
Citric acid ( $COOH-C(OH)(CH_2COOH)_2$   
Lactic acid ( $CH_3-CH(OH)-COOH$   
Hydroxy isobutyric acid ( $CH_3$ )<sub>2</sub>-C(OH)-COOH  
Levulinic acid  $CH_3CO-(CH_2)_2-COOH$

Esters derived from the first group of acids are characterized as follows on the basis of gas and carbon formation as compared to equivalent arcing in the mineral oil normally used in contactors and switches (mineral oil=100).

|                 | Per cent |
|-----------------|----------|
| Gas formed      | 50-60    |
| Carbon formed   | 20-50    |
| Carbon settling | 0        |

Esters derived from the acids of the second group are characterized as follows on the basis of gas and carbon formation as compared to equivalent arcing in the mineral oil normally used in contactors and switches (mineral oil=100).

|                 | Per cent |
|-----------------|----------|
| Gas formed      | 25-40    |
| Carbon formed   | 10-20    |
| Carbon settling | 0        |

It is not necessary that the alkyl esters should be used singly. It is possible, and even preferable in order to obtain the desired physical properties, such as a low freezing point, which is necessary for certain out-of-doors locations, to mix esters of different chemical formulation. Illustrative of such mixtures are compositions of ethyl and butyl citrate. A solution composed of equal proportions by weight of these esters has a freezing point of  $-40^{\circ}C$ . When subjected to the electric arc such a blend or solution evolves about

40 per cent as much gas as does the usual switch mineral oil and forms only about 16 per cent as much carbon which shows substantially no tendency to settle.

- 5 In like manner, the benefits of this invention may be obtained by blending alkyl esters with mineral oil. In general, the advantages thereby obtained are in proportion to the amount of ester composition present. For example, in a liquid composition consisting of 50 parts by weight each of dibutyl sebacate and the usual switch or contactor oil, the gas and carbon formed on arcing is about one-half that normally expected from the mineral oil itself. Surprisingly, substantially 10 no carbon settles from such solution after having been subjected to arcing and the behavior practically duplicates the non-settling characteristic already described in connection with a quenching medium consisting of dibutyl sebacate.
- 15 The advantages of my invention can be illustrated with reference to the five types of organic esters which have been found to be particularly advantageous. These include butyl lactate, butyl sebacate and butyl oxalate, and ethyl hydroxy isobutyrate. Butyl lactate and ethyl hydroxy isobutyrate represent esters derived from hydroxy monocarboxylic acids (propionic and butyric). Butyl oxalate represents an ester derived from a polycarboxylic acid (oxalic acid). Butyl sebacate represents an ester derived from a polycarboxylic acid. A mixture of equal parts by weight of ethyl and butyl citrate, and esters derived from a polycarboxylic hydroxy acid (citric acid) is an advantageous arc-quenching medium.

20 The following results obtained with an electrical contactor arranged to operate at 250 volts breaking a current of  $2\frac{1}{2}$  amperes 24 times a minute for three hours illustrate the advantages of my invention. At the end of this period of operation examination was made of the carbon formed and the rate of carbon settling. To do this, the arced liquid was well mixed and 50 milliliters were taken for examination. The amount of carbon was gravimetrically determined. Samples of the arced liquid were then set aside in tall cylinders at  $25^{\circ}C$ . for five hours and the amount of carbon which had settled from the top 25 per cent of the liquid was determined. The results obtained are listed below. In this tabulation, the relative amount of carbon, carbon settling and gas formed in mineral switch oil is given as 100:

| Carbon formed             |     |
|---------------------------|-----|
| Mineral switch oil        | 100 |
| Butyl sebacate            | 16  |
| Butyl lactate             | 11  |
| Ethyl hydroxy isobutyrate | 13  |
| Ethyl and butyl citrate   | 16  |
| Butyl oxalate             | 12  |

| Carbon settled in five hours |     |
|------------------------------|-----|
| Mineral switch oil           | 100 |
| Butyl sebacate               | 0   |
| Butyl lactate                | 0   |
| Ethyl hydroxy isobutyrate    | 0   |
| Ethyl and butyl citrate      | 0   |
| Butyl oxalate                | 0   |

| Gas formed                |     |
|---------------------------|-----|
| Mineral switch oil        | 100 |
| Butyl sebacate            | 18  |
| Butyl lactate             | 40  |
| Ethyl hydroxy isobutyrate | 40  |
| Ethyl and butyl citrate   | 17  |
| Butyl oxalate             | 17  |

As already stated, the liquid esters of the mono-carboxylic acids are suitable for the purposes of my invention. When tested as described in the foregoing paragraphs, the esters of oleic and of stearic acid such as methyl stearate, amyl oleate and butyl laurate give the following advantageous results:

*Carbon formed*

|                    |     |    |
|--------------------|-----|----|
| Mineral switch oil | 100 | 10 |
| Amyl oleate        | 34  |    |
| Butyl laurate      | 26  |    |
| Methyl stearate    | 24  |    |

*Carbon settled in five hours*

|                    |     |    |
|--------------------|-----|----|
| Mineral switch oil | 100 | 15 |
| Amyl oleate        | 0   |    |
| Butyl laurate      | 0   |    |
| Methyl stearate    | 0   |    |

*Gas formed*

|                    |     |    |
|--------------------|-----|----|
| Mineral switch oil | 100 | 20 |
| Amyl oleate        | 50  |    |
| Butyl laurate      | 45  |    |
| Methyl stearate    | 48  |    |

In general, an arc-quenching liquid should have a viscosity not exceeding about 150 seconds Saybolt Universal at 37.8° C. (100° F.). The characteristics of several typical ester compositions used in combination with contactors and liquid-filled electrical switching devices in accordance with my invention are:

|                | Specific Gravity 15.6° C. | Viscosity Saybolt Universal Seconds at 37.8° C. | Fire Point | Pour Point ° C. |
|----------------|---------------------------|-------------------------------------------------|------------|-----------------|
| Butyl sebacate | .940                      | 46                                              | 208        | -10             |
| Amyl oxalate   | .970                      | 56                                              | 126        | -22             |
| Amyl oleate    | .862                      | 47                                              | 205        | -12             |
| Butyl laurate  | .855                      | 39                                              | 165        | -13             |
| Butyl stearate | .858                      | 48                                              | 208        | 20              |

What I claim as new and desire to secure by Letters Patent of the United States is:

1. An electric circuit-interrupter containing separable electric contacts and an arc-quenching liquid operatively associated with said contacts, said liquid consisting of a substantially water-insoluble alkyl ester of aliphatic acid in which the organic acid radical contains from two to eighteen carbon atoms, and the ester alkyl radical contains one to five carbon atoms.

2. An electric circuit interrupter comprising make-and-break contacts and a water-insoluble liquid-quenching medium, the active agent of said medium consisting exclusively of an alkyl compound of an aliphatic acid containing from two to eighteen carbon atoms and being chosen from a group consisting of monocarboxylic acids, carboxylic acids containing respectively a hy-

droxy or ketone group and carboxylic acids containing a plurality of carboxy groups.

3. An electric circuit-interrupter containing separable arcing contacts and an arc-quenching liquid enveloping said contacts, said liquid consisting of mineral oil and a water-insoluble alkyl ester in which the alkyl radical contains one to five carbon atoms and the acid radical contains 2 to 18 carbon atoms.

4. An electric circuit-interrupter containing separable arcing contacts and an arc-quenching liquid enveloping said contacts, said liquid consisting exclusively of an alkyl ester of hydroxy monocarboxylic acid, the ester alkyl radical of which contains one to five carbon atoms and the acid radical of which contains two to eighteen carbon atoms, said ester having a viscosity not exceeding 150 seconds Saybolt at 37.8° C.

5. An electric circuit-interrupter containing separable arcing contacts and an arc-quenching liquid enveloping said contacts, said liquid consisting of an alkyl ester of polycarboxylic acid, the ester alkyl radical of which contains one to five carbon atoms and the acid radical of which contains two to eighteen carbon atoms, said ester having a viscosity not exceeding 150 seconds Saybolt at 37.8° C.

6. An electric circuit-interrupter containing separable arcing contacts and an arc-quenching liquid enveloping said contacts, said liquid consisting of mineral oil and dibutyl sebacate.

7. An electric circuit-interrupter containing separable arcing contacts and an arc-quenching liquid enveloping said contacts, said liquid consisting of substantially equal parts by weight of mineral oil and dibutyl sebacate.

8. An electric circuit-interrupter containing separable arcing contacts and an arc-quenching liquid enveloping said contacts, said liquid consisting exclusively of alkyl ester of citric acid, the alkyl radical of said ester containing one to five carbon atoms.

9. An electric circuit-interrupter containing separable arcing contacts and an arc-quenching liquid enveloping said contacts, said liquid consisting exclusively of a mixture of equal parts by weight of ethyl and butyl citrate.

10. An electric circuit-interrupter containing separable arcing contacts and an arc-quenching liquid enveloping said contacts, said liquid consisting of dibutyl sebacate.

FRANK M. CLARK.

REFERENCES CITED

55 The following references are of record in the file of this patent:

FOREIGN PATENTS

60 Number Country Date  
682,816 Germany Oct. 24, 1939